

## UNITED STATES PATENT OFFICE

JEFFREY DENNISS AND THOMAS REID, OF SYDNEY, NEW SOUTH WALES,  
AUSTRALIA

## TANNING HIDES AND SKINS

No Drawing. Application filed November 29, 1929, Serial No. 410,634, and in Australia January 21, 1929.

This invention concerns a process for tanning animal hides and skins, in which the cost of production is low and the time required for manufacture is considerably less than in existing methods, while a leather of excellent wearing qualities without the objectionable odour which so frequently accompanies tanned goods is produced.

After the usual preliminary softening and plumping treatment, the hides or skins in wet condition are placed in vacuo, or in partial vacuo—which should not be less than 14½ lbs. sub-atmosphere—for about six to twelve hours, and then lime liquor is introduced into the vacuum chamber. They remain submerged in the lime liquor until fit for de-hairing, about five or six days and they are then washed to remove lime. Next follows the usual beam-house treatment, at the conclusion of which they are immersed in liquor of strength about 12° barkometer for a period of one to two days. Thereafter the hides or skins are hung or packed in layers with ground tan bark and covered with tan vegetable liquor in specially constructed tan pits; these pits are enclosed and they are held in a state of vacuum as complete as practicable for a period of two days. After this vacuum treatment the pelts are immersed in pure concentrated tan vegetable liquor not less than 50° barkometer in strength, and according to their substance are retained therein from ten to thirty-five days. The leather thus produced is subjected to the usual finishing operations and may be dyed to bring it to any colour desired.

The fibre becomes tightened up in the process, even on the loosest belly pieces, and a firm tough leather having good wearing properties is obtained.

Loss in weight during the process, due to corrosion and solution of the hides or skins is low. The wearing qualities of the product are not diminished as in most known quick tanning processes.

What we claim as our invention and desire to secure by Letters Patent is:—

A process of tanning hides and skins, comprising the sequential steps of preliminarily softening and plumping the hides, maintain-

ing the hides in vacuum for from 6 to 12 hours; liming the hides for from 5 to 6 days, de-hairing, de-liming, and beaming the hides, immersing the hides in tan liquid at approximately 12° barkometer from 1 to 2 days; 55 packing the hides in tan bark in vacuum for approximately 2 days; immersing the hides in tan liquor for approximately 10 days to 35 days; and finishing the hides; the periods of treatment being varied with regard to the 60 substance of the hides under treatment.

In testimony whereof we affix our signatures.

JEFFREY DENNISS.  
THOMAS REID.

65

70

75

80

85

90

95

100